

## UNITED STATES PATENT OFFICE

JOSEPH KENT SMITH, OF DETROIT, MICHIGAN, ASSIGNOR TO BERYLLIUM DEVELOPMENT CORPORATION, OF NEW YORK, N. Y., A CORPORATION OF DELAWARE

## BERYLLIUM-ALUMINUM ALLOY

No Drawing.

Application filed December 22, 1931. Serial No. 582,657.

- This invention relates to alloys characterized by extreme lightness and great strength, having metallic beryllium as the predominating component of the alloy.
- 5 Inasmuch as elementary beryllium in unalloyed form tends to great brittleness, and therefore cannot readily be rolled, forged, or subjected to those other mechanical operations necessary to bring metals into readily-usable forms, especially those forms used where extreme lightness is required, it has been found necessary to alloy beryllium with smaller quantities of aluminum so as to obtain an ultra-light metallic material possessing those characteristics which will permit of the mechanical operations cited. The proportions of aluminum added to the beryllium will vary in quantity with the requirements of the situation, the lower the quantity of 10 aluminum added, the lighter the resulting alloy, but correspondingly greater are the difficulties of mechanical manipulation. When the aluminum content of the alloy is as little as ten percent of the total, great precautions are necessary in rolling or forging the alloy, while the alloy with thirty percent of aluminum, with a specific gravity of approximately 2.0, lends itself quite readily to all the usual methods of mechanical treatment. Alloys of about equal parts of beryllium and aluminum are still easier to work, but they lack the greater strength and superior lightness of the alloys lower in aluminum. The alloy approximating seventy 15 percent beryllium and thirty percent aluminum represents best current practice in this series, presenting a nice balance between the various factors involved.
- However, the simple binary beryllium-aluminum alloys, despite their greater strength as compared with pure aluminum, leave much to be desired in the matter of strength, machinability, resistance to corrosion, etc. I have found, in my invention, that 20 by adding, to any of the beryllium-aluminum alloy series in which beryllium predominates, small quantities of manganese and zirconium, with or without simultaneous additions of small quantities of molybdenum, significant increases in strength, machinability, resistance to corrosive influences, etc., can be effected, without any material increase in the specific gravity of the alloy. The "heavy" metals mentioned as addition agents—manganese, zirconium, molybdenum—should never exceed five percent of the total weight of the alloy, and, in the preferred compositions, these metals do not exceed two percent of the total.
- If desired, such alloys can be made by the addition of the requisite quantities of the free heavy metals to a molten beryllium-aluminum alloy. The zirconium can also be added in the form of the carbon-free zirconium-aluminum alloy which is so readily made by the reduction of zirconium oxide with aluminum. Another method consists in melting the beryllium and aluminum together first, employing as a flux a mixture of the chlorides and fluorides of calcium with some cryolite. To this, the zirconium (and, if desired, the molybdenum) is added in the form of compounds easily reducible in the circumstances, like zirconium, dioxide or calcium zirconate (and calcium molybdate). Under the conditions, elementary zirconium (and molybdenum) is formed by reduction and enters into the alloy. The manganese is added then by means of a cleansing alloy, comprising aluminum, magnesium and manganese. The magnesium almost all boils out readily, while the manganese and aluminum unite with the primary alloy, resulting in the final multi-constituent alloy.
- As compared with the simple binary beryllium-aluminum alloy of seventy percent beryllium content, a similar alloy containing about one-half percent each of zirconium, molybdenum and manganese is more readily workable, flows better, casts better, has greater strength and resistance to corrosion, and is more readily flexed without cracking. In sheet form, say from fifteen to twenty thousandths of an inch in thickness, a strength of one hundred to one hundred and ten thousand pounds to the square inch is obtained. In such sheet form, the alloy is particularly useful for airplane wings and fuselage parts, or wherever else the combination of ultra-lightness and strength is required.

lightness, strength and bendability without breaking is essential.

The presence of the heavy metals hardens the aluminum eutectic, giving the multi-constituent alloy a relatively low coefficient of friction. The alloy is, therefore, useful for piston rings, pistons, and similar moving parts involving frictional effects.

In cast form, alloys covered by this invention have tensile strengths ranging from thirty thousand to fifty thousand pounds per square inch.

While I prefer approximately 70% beryllium content, the invention is applicable with approximately the following composition: beryllium from about 55% to about 70%, aluminum from about 25% to about 40%, with the manganese, zirconium and molybdenum, if used, making up the balance in approximately equal amounts.

A preferred analysis is:—

|              | Per cent |
|--------------|----------|
| Be           | 69.4     |
| Al           | 29.0     |
| 25 Mn        | .6       |
| Zr           | .3       |
| Mo           | .5       |
|              | <hr/>    |
| 30 Mg. added | .7       |
|              | 99.8     |

The percentages are by weight.

I claim:—

1. A beryllium-aluminum alloy of approximately the following composition: beryllium from about 55% to about 70%, aluminum from about 25% to about 40% and manganese, molybdenum and zirconium in approximately equal amounts from about  $\frac{1}{2}\%$  to about  $2\frac{1}{2}\%$  each.

2. A beryllium-aluminum alloy of approximately the following composition: beryllium from about 55% to about 70%, aluminum from about 25% to about 40%, and manganese, molybdenum and zirconium from about  $\frac{1}{2}\%$  to about  $2\frac{1}{2}\%$  each but not approximately in excess of 5% in the aggregate.

In testimony whereof I have hereunto signed my name.

JOSEPH KENT SMITH.